# EUROPEAN PATENT SPECIFICATION

(11) **EP 3 312 340 B1**
(45) Date of publication and mention of the grant of the patent: **28.07.2021**
(21) Application number: 15896383.5
(22) Date of filing: 26.06.2015
(51) Int. Cl.: D21H 27/00, A24D 1/02, D21H 25/00, D21H 17/67

(54) **CIGARETTE PAPER, MANUFACTURING METHOD AND MANUFACTURING DEVICE THEREOF, AND CIGARETTE**
ZIGARETTENPAPIER, HERSTELLUNGSVERFAHREN UND HERSTELLUNGSVORRICHTUNG DAFÜR UND ZIGARETTE
PAPIER DE CIGARETTE, PROCÉDÉ DE FABRICATION ET DISPOSITIF DE FABRICATION DE CELUI-CI, ET CIGARETTE

(43) Date of publication of application: 25.04.2018
(62) Divisional of application: 20170037.4
(73) Proprietor: JAPAN TOBACCO INC., Minato-ku Tokyo 105-8422 (JP)
(72) Inventor: KITAOKA, Ryo, Tokyo 130-8603 (JP); YOSHIMURA, Tetsuya, Tokyo 130-8603 (JP)
(74) Representative: Hoffmann Eitle
(86) International application number: PCT/JP2015/068521
(87) International publication number: WO 2016/208065

(56) References cited:
- WO-A1-97/09483
- CN-A- 101 935 962
- JP-A- H0 949 198
- JP-A- S5 529 955
- JP-A- H05 279 983
- JP-A- H08 246 396
- US-A1- 2009 301 506
- US-A1- 2012 227 754
- None

## Description

### Technical Field

The present invention relates to cigarette paper, a method and an apparatus for making same, and a cigarette.

### Background Art

In the field of papermaking, calendering is publicly known as disclosed in Patent Documents 1 and 2 identified below. Soft calendering of Patent Document 1 is used to improve gloss and smoothness of a paper web without reducing its bulk, while calendering of Patent Document 2 is used to form a laminate from a metal foil strip and a paper strip.

### Prior Art Document

### Patent Document

Patent Document 1: International Application Japanese Translation Publication No. 2003-520910 (WO01/055505)
Patent Document 2: Japanese Unexamined Patent Application Publication No. Hei 6-344462 (US 5,169,481)
US 2012/227754 discloses a method for producing a cigarette paper comprising a calendering step.
US2009/301506 discloses a method for producing a cigarette paper comprising a calendering step and a low ignition cigarette paper produced by this method.

### Summary of the Invention

### Problems to be solved by the Invention

The calendering of Patent Document 1 is suitable for offset printing papers, but not suitable for cigarette papers which are thin as compared with such printing papers. A laminate formed by the calendering of Patent Document 2 is used to form tubular members for non-combustion smoking articles, and thus, not usable as cigarette paper which is to be burned.

Further, neither Patent Document 1 nor 2 discloses or suggests a calendering process which allows relatively thin cigarette paper to have a glossiness of at least 10% or higher.

An object of the present invention is to provide cigarette paper having a glossiness of at least 10% or higher, and a method and an apparatus for making same.

### Means for Solving the Problems

The above object is achieved by the method of claim 1. The preferred embodiments are described in the further claims.

The present description also provides an apparatus for making cigarette paper, which comprises
a traveling path along which a paper web containing a filler for increasing gloss is caused to travel, and
a processing section arranged on the traveling path to supercalender the paper web, thereby forming the paper web into cigarette paper, wherein the processing section is adapted to perform supercalendering under processing conditions that allow the cigarette paper to have glossiness of at least 10% or higher,
wherein the cigarette paper is 20 to 100µm, and
the filler is contained in the paper web in the amount exceeding at least 10gsm, and the paper web has a basis weight of 40 to 63gsm.

The present invention further provides a cigarette comprising cigarette paper having glossiness of at least 10% or higher.

### Advantageous Effects of the Invention

The method for making cigarette paper according to the present invention can make cigarette paper having glossiness of at least 10% or higher. The present invention can also provide a cigarette comprising such cigarette paper.

### Brief Description of the Drawings

FIG. 1 is a schematic front view of a cigarette paper making apparatus according to an embodiment of the present invention.
FIG. 2 is a schematic side view showing a processing section of the making apparatus of FIG. 1.
FIG. 3 is a graph showing the relation between filler content and glossiness on supercalendered cigarette paper.
FIG. 4 is a graph showing the results of sensory evaluation in which grade of supercalendered cigarette papers was evaluated based on their whiteness and the glossiness.
FIG. 5 shows a scale used in sensory evaluation.
FIG. 6 is a graph showing the results of sensory evaluation in which grade of supercalendered cigarette papers was evaluated based on their opacity and glossiness.
FIG. 7 is a graph showing the results of sensory evaluation in which feel of supercalendered cigarette papers was evaluated based on their smoothness.
FIG. 8 is a picture showing how a filtered cigarette comprising non-supercalendered cigarette paper burns, when left after ignited.
FIG. 9 is a picture showing how a filtered cigarette comprising supercalendered cigarette paper burns, when left after ignited.

### Mode of Carrying out the Invention

A cigarette paper making method according to an embodiment of the present invention is carried out by a making apparatus shown in FIGS. 1 and 2. First, the making apparatus will be outlined below.

The making apparatus comprises a traveling path 10 for a paper web W. The traveling path 10 extends from a feed roll R1 to a wind-up roll R2, for example horizontally. The paper web W can be fed from the feed roll R1 and wound onto the wind-up roll R2.

The making apparatus further comprises a calendering section 12. The calendering section 12 comprises a roller set 14. The roller set 14 includes a metal roller, which is, for example a steel roller 16, and a resin roller 18. The resin roller 18 is arranged below the traveling path 10, while the steel roller 16 is arranged immediately above the traveling path 10. The traveling path 10 thus is sandwiched between the steel roller 16 and the resin roller 18. The steel roller 16 is made of steel, while the resin roller 18 has an outer cylindrical surface formed of a synthetic resin coating. The hardness of the resin roller, which means the surface hardness of the coating of the resin roller 18, is between D-50 and D-120, preferably between D-80 and D-100 in durometer values. The durometer value is obtained by the measuring method specified in JIS K6253.

As indicated by broken lines in FIG 1, the steel roller 16 as well as the resin roller 18 has an electric heater 20 within themselves. The electric heaters 20 are electrically connected to a power supply (not shown). The power supply can maintain the temperatures of the outer cylindrical surfaces of the steel and resin rollers 16, 18, referred to as "roller temperatures", at a set value by means of the heaters 20. The set value for roller temperature is selected in the range of 25 to 160°C.

As seen in FIG. 2, in the present embodiment, the making apparatus further comprises a drive source 22 for rotating the steel roller 16 in one direction and an elevating mechanism 24 for moving up and down the resin roller 14 relative to the steel roller 16.

The drive source 22 includes a drive motor 26. The drive motor 26 is connected to a roller shaft of the steel roller 16 by means of a pair of power transmission gears 28. The drive source 22 further includes a speed regulator 30 electrically connected to the drive motor 26. The speed regulator 30 can regulate the circumferential speed of the steel roller 16 to a set value by means of the drive motor 26.

The elevating mechanism 24 includes a pair of hydraulic cylinders 32. The hydraulic cylinders 32 are connected to the opposite ends of a roller shaft of the resin roller 18, respectively. The hydraulic cylinders 32 are connected to a hydraulic pressure source (not shown) including a hydraulic pump. The hydraulic pressure source controls supply and discharge of a hydraulic fluid to and from the respective hydraulic cylinders 32. The hydraulic pressure source can thus move up and down the resin roller 18 while maintaining it in a horizontal position. Thus, the paper web W traveling on the traveling path 10 is compressed as it passes between the steel roller 16 and the resin roller 18.

Further, the elevating mechanism 24 includes pressure regulation valves (not shown) assigned to the respective hydraulic cylinders 32. The pressure regulation valves regulate the pressure applied to the steel roller 16 by the resin roller 18. The pressure regulation valves can thus regulate the compressive pressure applied to the paper web W to a set value. In the present embodiment, the pressure regulation valves are operated manually. FIG. 2 shows operating handles 34 for the pressure regulation valves arranged near the respective hydraulic cylinders 32.

Further, temperature sensors 36 are provided to the steel roller 16 and the resin roller 18 to measure the roller temperatures, while pressure sensors 38 are provided to the respective hydraulic cylinders 32 to measure the compressive pressures (linear pressures) applied to the paper web W.

In the making method using the above-described making apparatus, a paper web W is fed from the feed roll R1, where the paper web has desirably a moisture content of 3 to 7wt%. The moisture content is obtained by the measuring method specified in JIS P8123. The paper web W fed passes through the calendering section 12 while sandwiched between the steel roller 16 and the resin roller 18. The steel roller 16 and the resin roller 18 compress the paper web W. In the present making method, the paper web W is supercalendered in this manner, and then, the calendered paper web W is wound onto the wind-up roll R2.

Here, it is to be noted that in the present embodiment, the paper web W is supercalendered with its top side and back side in contact with the resin roller 18 and the steel roller 16, respectively.

In the present embodiment, the paper web W is formed from a pulp material suited for cigarette paper in a paper machine. The paper web W has a basis weight of 40 to 63gsm, optionally an apparent density of 600 to 900kg/m³. Such paper web is formed into cigarette paper by the above-described supercalendering. In other words, the paper web W wound onto the roll R2 is used as cigarette paper to make cigarettes. For example, FIG. 1 shows a cigarette, specifically a filtered cigarette FC. The filtered cigarette FC comprises a length of cigarette paper CP. Such cigarette paper CP is 20 to 100µm thick, preferably 30 to 90µm thick.

Supercalendering increases the apparent density of the paper web W. It gives an apparent density of 800 to 1500kg/cm³, preferably 1000 to 1300kg/cm³ to the paper web W. Tensile force applied to the paper web W in supercalendering only needs to be at a level that the paper web W can withstand. For example, the tensile force is 20.0N/15mm or less, preferably 12.5N/15mm or less.

In the present embodiment, the paper web W contains a filler which is effective in improving gloss of the cigarette paper CP in cooperation with supercalendering. Here, the filler includes calcium carbonate.

To validate the gloss improving effect of the filler, paper webs W having differing filler contents were prepared. Those paper webs W were superecalendered under specified processing conditions. The results of validation test are shown in FIG. 3. FIG. 3 shows the relation between filler content and glossiness of cigarette paper CP.

In FIG. 3, marks ○, Δ, □ represent cases in which paper web W was supercalendered under differing processing conditions, or in other words, with differing hardness (D-XX) of the resin roller 18 and differing roller temperature (°C). Mark ◊ represents cases in which paper web W was not supercalendered. The hardness of the resin roller 18 is expressed in aforementioned durometer values.

The results of validation test shown in FIG. 3 were obtained with the other processing conditions fixed. Specifically, the traveling speed of paper web W and the compressive pressure (linear pressure) were fixed at 5m/min and 5.6 N/mm, respectively. Incidentally, the traveling speed of paper web W and the compressive pressure may be set appropriately. For example, the traveling speed is selected within the inventive range of 3 to 1000m/min, and the compressive pressure is selected within the inventive range of 3 to 10N/mm.

The glossiness of cigarette paper CP was obtained by the measuring method specified in JAPAN TAPPI (the Technical Association of the Pulp and Paper Industry) No. 72.

The filler content was measured by the measuring method described below.

First, a solution that can dissolve the filler (an acidic solution or a basic solution, for example) is prepared. Then, paper web W is immersed in the solution to cause all the filler to transfer from the paper web W into the solution. Then, the amount of the filler in the solution is measured by an analytical instrument based on capillary electrophoresis or gas-chromatography.

With regard to the glossiness of cigarette paper CP, FIG. 3 shows the following:
(i) With regard to cigarette paper CP not subjected to supercalendering (see ◊), an increase in filler content does practically not increase the glossiness of cigarette paper CP.
(ii) Supercalendering with higher filler content increases the glossiness of cigarette paper CP to greater extent.
(iii) Provided that the roller temperature is the same, supercalendering with higher hardness of the resin roll 18 increases the glossiness of cigarette paper CP to greater extent.
(vi) Provided that the hardness of the resin roll 18 is the same, supercalendering at higher temperature of the resin roll 18 increases the glossiness of cigarette paper CP to greater extent.

Accordingly, in order to increase the glossiness of cigarette paper CP, it is necessary to increase the filler content or make the processing conditions concerning the roller temperature and hardness of the resin roll 18 harsher for the paper web W. For example, as seen from FIG. 3, if the cigarette paper CP needs to have glossiness of 10% or higher, the filler content needs to exceed at least 10gsm, and in order to give the cigarette paper CP glossiness of 15% or higher, the filler content needs to exceed at least 20gsm. However, too high filler content may lead to decreased tensile strength of the paper web W. Thus, the filler content is desirably higher than 20gsm and lower than 50gsm.

The inventors have confirmed that with regard to variations in glossiness of cigarette paper CP, the same tendency as seen in FIG. 3 is observed with different types of paper webs W. This has been confirmed with four types of paper webs indicated in Table 1 below

**[Table 1]**

| W | Pulp type | Basis weight [gsm] | Filler content [gsm] | Pulp content [gsm] |
|---|---|---|---|---|
| #1 | Wood | 62.7 | 29.9 | 32.8 |
| #2 | Wood | 47.4 | 23 | 24.4 |
| #3 | Flax | 32 | 8.3 | 23.7 |
| #4 | Flax | 26 | 8.3 | 17.7 |

Table 2 below shows the relation between pulp type and glossiness and smoothness of cigarette paper CP.

**[Table 2]**

| W | Pulp type | Basis weight [gsm] | Pulp content [gsm] | Filler content [gsm] | Hardness | Roller temperature [°C] | Glossiness [%] | Smoothness [s] |
|---|---|---|---|---|---|---|---|---|
| #5 | Flax | 23.5 | 16.8 | 6.7 | - | - | 5.1 | 49.8 |
| | | | | | D-83 Resin | 25 | 11.4 | 99.6 |
| | | | | | | 80 | 16.1 | 433 |
| #6 | Wood | | 16.2 | 7.3 | - | 25 | 5.7 | 137.9 |
| | | | | | D-83 Resin | | 11.4 | 450.6 |
| | | | | | | 80 | 15.8 | 480.5 |

Table 3 below shows the relation between pulp content and glossiness and smoothness of cigarette paper CP.

**[Table 3]**

| W | Pulp type | Basis weight [gsm] | Pulp content [gsm] | Filler content [gsm] | Hardness | Roller temperature [°C] | Glossiness [%] | Smoothness [s] |
|---|---|---|---|---|---|---|---|---|
| #3 | Flax | 32 | 23.7 | 8.3 | - | - | 4.1 | 20.1 |
| | | | | | D-83 Resin | 25 | 9.6 | 210.1 |
| | | | | | | 80 | 14.2 | 320 |
| #4 | | 26 | 17.7 | | - | 25 | 4.6 | 58.9 |
| | | | | | D-83 resin | | 9.4 | 275.7 |

In Tables 2 and 3, the sign "-" in the "Hardness" column indicates that supercalendering was not performed.

As is clear from Table 2, glossiness of cigarette paper CP does practically not vary with differing pulp type. Further, as is clear from Table 3, glossiness of cigarette paper CP does practically not vary with differing pulp content.

When calcium carbonate is added as a filler, it is known that calcium carbonate increases whiteness and opacity of a paper web W, and thus, of cigarette paper CP. Whiteness and opacity as well as glossiness serve as an index of grade of cigarette paper CP.

FIG. 4 shows the results of sensory evaluation in which eleven assessors evaluated grade of each paper web CP based on glossiness and whiteness. The scale used in the sensory evaluation is shown in FIG. 5. FIG. 4 shows that cigarette paper CP with glossiness of 10% or higher and with whiteness of 88 to 90 gives an impression of "high grade", where the glossiness of cigarette paper CP is preferably 15 to 40%. The whiteness of cigarette paper CP was measured by the measuring method specified in JIS P 8148-2001 (ISO 2470).

Sensory evaluation of grade of cigarette paper CP can be made based on glossiness and opacity in place of whiteness. The results of sensory evaluation made this way are shown in FIG. 6. Also in this sensory evaluation, the scale shown in FIG. 5 was used.

FIG. 6 shows that cigarette paper CP with glossiness of 10% or higher and with opacity of 82 to 92, or in other word, at least 82 or higher gives an impression of "high grade". The opacity of cigarette paper was measured by the measuring method specified in ISO 2471.

Further, supercalendering increases smoothness of cigarette paper CP. Sensory evaluation of feel of cigarette paper CP can be made based on smoothness using the scale shown in FIG. 5. The results of evaluation made this way are shown in FIG. 7. The smoothness of cigarette paper CP was measured by the measuring method specified in JIS P 8119 (ISO 5627). FIG. 7 shows that cigarette paper with a smoothness of 400" or higher, preferably 700" or higher gives a good feel. Increase in smoothness of cigarette paper CP is also effective in reducing paper dust produced from cigarette paper CP in the process of making filtered cigarettes. Further, increase in smoothness of cigarette paper CP is also effective in increasing ease of removing a filtered cigarette FC from a cigarette package. Too high smoothness of cigarette paper CP may cause a slip of cigarette paper CP in the wrapping process, or process of wrapping smokable materials including tobacco shreds with the cigarette paper CP, which may lead to reduced productivity in making cigarette rods, and thus, making cigarettes. As a result, the smoothness of cigarette paper CP is desirably 3000" or lower, for example.

Supercalendering increases the density of cigarette paper CP, and thus, is effective in suppressing flying of ash produced by smoking a filtered cigarette comprising cigarette paper CP.

FIG. 8 shows how a filtered cigarette made using a paper web W (#1) not subjected to supercalendeing burns, when left after ignited, and FIG. 9 shows how a filtered cigarette FC made using cigarette paper CP formed by supercalendering a paper web W (#1) burns, when left after ignited, where supercalendering was performed under conditions of resin roll hardness D-90 and roller temperature 80 °C. Comparison between FIGS. 8 and 9 shows that the filtered cigarette comprising supercalendered cigarette paper produces a stable mass of ash, so that flying of ash is effectively suppressed.

Further, supercalendering, which increases the density of cigarette paper CP, reduces the burning rate of the cigarette paper CP, reduces minute pin holes in the cigarette paper CP and reduces the air permeability of the cigarette paper CP. Controlling of burning rate serves to provide a required appropriate number of puffs per filtered cigarette FC. Here, the controlling is effective when cigarette paper CP not subjected to supercalendering has too high a burning rate to provide an appropriate number of puffs per filtered cigarette FC. Reduction of minute pin holes serves to reduce the amount of visible sidestream smoke from a filtered cigarette FC, and reduction of air permeability serves to improve a sensation of resistance caused by drawing on a filtered cigarette FC at initial puffs.

The present invention is not restricted to the described embodiment but may be altered in various ways. For example, a filler for improving gloss of cigarette paper CP other than calcium carbonate may be used in combination with calcium carbonate. It goes without saying that the processing conditions for supercalendering other than those concerning the hardness of the resin roller 18 and the roller temperature may be varied. For example, the traveling speed of the paper web W and the compressive pressure applied to it may be varied appropriately.

The cigarette diameter representing the transverse size (cross-sectional area) of the filtered cigarette FC comprising cigarette paper CP according to the present invention is not restricted to a specified value. Ordinary cigarettes have a diameter of 7.5 to 8.5mm. Among slim-sized cigarettes smaller in diameter than ordinary cigarettes, there are known cigarettes with a diameter of 6.5 to 7.5mm and cigarettes with a diameter of 5.0 to 6.5mm. Thus, the diameter of the cigarette according to the present invention may be selected in the range of 5.0 to 8.5mm. However, the consumer's perceived glossiness of cigarette paper CP depends on the angular displacement of the consumer's line of sight. Cigarette of smaller diameter, or in other words, cigarette circumference of greater curvature results in greater angular displacement of the consumer's line of sight per unit length of cigarette circumference, so that the consumer perceives higher glossiness of cigarette paper.

### Explanation of Reference Signs

- 10: Traveling path
- 12: Processing section
- 14: Roller set
- 16: Steel roller (metal roller)
- 18: Resin roller
- 20: Electric heater
- 22: Drive source
- 24: Elevating mechanism
- 36: Temperature sensor
- 38: Pressure sensor
- W: Paper web
- CP: Cigarette paper
- FC: Filtered cigarette

## Claims

1. A method of making cigarette paper (CP), comprising
causing a paper web (W) containing a filler for increasing gloss to travel, and
supercalendering the traveling paper web (W), thereby forming the paper web (W) into cigarette paper (CP), wherein supercalendering is performed under processing conditions that allow the cigarette paper (CP) to have glossiness of at least 10% or higher, measured according to JAPAN TAPPI No. 72,
wherein the traveling speed of the paper web (W) is selected within the range of 3 to 1000m/min and
the filler includes calcium carbonate and
the cigarette paper is 20 to 100µm thick, and
the filler is contained in the paper web in the amount exceeding at least 10gsm and lower than 50gsm and the paper web has a basis weight of 40 to 63gsm,and
the paper web (W) is supercalended by a roller set (14) including a metal roller (16) and a resin roller (18) which applies compressive pressure to the paper web (W) passing between the metal roller (16) and the resin roller (18) and
the processing conditions include conditions concerning roller temperature of the roller set (14) and the compressive pressure and
the roller temperature is selected in the range of 25 to 160°C, and
the compressive pressure is selected within the range of 3 to 10N/mm.

2. The method of making cigarette paper (CP) according to claim 1, wherein
the processing conditions include condition concerning hardness of the resin roller (18).

3. The method of making cigarette paper (CP) according to claim 2, wherein the filler is a substance which increases not only gloss but also opacity of the cigarette paper (CP).

4. A cigarette comprising cigarette paper (CP) with glossiness of 10% or higher, measured according to JAPAN TAPPI No. 72,
wherein the cigarette paper (CP) is made by supercalendering a paper web (W) containing a filler for increasing gloss, the cigarette paper (CP) is 20 to 100µm thick and the filler includes calcium carbonate and,
the filler is contained in the paper web (W) in the amount exceeding at least 10gsm, and the paper web (W) has a basis weight of 40 to 63gsm.

5. The cigarette according to claim 4, wherein the cigarette paper (CP) has opacity of 82 or higher.

6. The cigarette according to claim 4, wherein the cigarette paper (CP) has smoothness of 400" or higher.

## Patentansprüche

1. Verfahren zur Herstellung von Zigarettenpapier (CP), umfassend
das Bewirken, dass eine Papierbahn (W) einen Füllstoff enthält, um Glanz zum Laufen zu erhöhen, und
Superkalandieren der laufenden Papierbahn (W), wodurch die Papierbahn (W) in Zigarettenpapier (CP) geformt wird, wobei Superkalandieren unter Verarbeitungsbedingungen durchgeführt wird, die es dem Zigarettenpapier (CP) ermöglichen, Glanz von mindestens 10% oder mehr, gemessen nach JAPAN TAPPI Nr. 72, aufzuweisen,
wobei die Laufgeschwindigkeit der Papierbahn (W) innerhalb des Bereichs von 3 bis 1000m/min ausgewählt wird, und
der Füllstoff Kalziumkarbonat beinhaltet, und
das Zigarettenpapier 20 bis 100µm dick ist, und
der Füllstoff in der Papierbahn in der Menge enthalten ist, die mindestens 10 g übersteigt, und niedriger als 50 g ist, und die Papierbahn ein Grundgewicht von 40 bis 63 g aufweist, und
die Papierbahn (W) durch einen Walzensatz (14) superkalandiert wird, der eine Metallwalze (16) und eine Harzwalze (18) beinhaltet, die einen Kompressionsdruck an die Papierbahn (W) anlegt, der zwischen der Metallwalze (16) und der Harzwalze (18) verläuft, und
die Verarbeitungsbedingungen Bedingungen hinsichtlich der Walzentemperatur des Walzensatzes (14) und des Kompressionsdrucks beinhalten,
und
die Walzentemperatur in dem Bereich von 25 bis 160°C ausgewählt wird,
und
der Kompressionsdruck innerhalb des Bereichs von 3 bis 10 N/mm ausgewählt wird.

2. Verfahren zur Herstellung von Zigarettenpapier (CP) nach Anspruch 1, wobei
die Verarbeitungsbedingungen eine Bedingung hinsichtlich der Härte der Harzwalze (18) beinhalten.

3. Verfahren zur Herstellung von Zigarettenpapier (CP) nach Anspruch 2, wobei der Füllstoff eine Substanz ist, die nicht nur Glanz, sondern auch Opazität des Zigarettenpapiers (CP) erhöht.

4. Zigarette, Zigarettenpapier (CP) mit Glanz von 10% oder mehr, gemessen nach JAPAN TAPPI Nr. 72, umfassend,
wobei das Zigarettenpapier (CP) durch Superkalandieren einer Papierbahn (W), die einen Füllstoff zum Erhöhen von Glanz enthält, hergestellt wird, wobei das Zigarettenpapier (CP) 20 bis 100µm dick ist, und der Füllstoff Kalziumkarbonat beinhaltet, und
der Füllstoff in der Papierbahn (W) in der Menge enthalten ist, die mindestens 10 g übersteigt, und die Papierbahn (W) ein Grundgewicht von 40 bis 63 g aufweist.

5. Zigarette nach Anspruch 4, wobei das Zigarettenpapier (CP) eine Opazität von 82 oder mehr aufweist.

6. Zigarette nach Anspruch 4, wobei das Zigarettenpapier (CP) eine Geschmeidigkeit von 400" oder mehr aufweist.

## Revendications

1. Procédé de fabrication de papier à cigarettes (CP), comprenant
l'activation du déplacement d'une bande de papier (W) contenant une charge pour augmenter la brillance, et
le satinage de la bande de papier (W) se déplaçant, formant ainsi la bande de papier (W) en papier à cigarettes (CP), dans lequel le satinage est effectué dans des conditions de traitement qui permettent au papier à cigarettes (CP) d'avoir une brillance d'au moins 10 % ou plus, mesurée selon la norme JAPAN TAPPI N°72,
dans lequel la vitesse de déplacement de la bande de papier (W) est choisie dans la plage allant de 3 à 1000 m/min. et
la charge inclut du carbonate de calcium et
le papier à cigarettes présente une épaisseur allant de 20 à 100 µm, et
la charge est contenue dans la bande de papier dans la quantité dépassant au moins 10 gsm et étant inférieure à 50 gsm et la bande de papier présente un poids de base allant de 40 à 63 gsm, et
la bande de papier (W) est satinée par un ensemble de rouleaux (14) incluant un rouleau en métal (16) et un rouleau en résine (18) qui applique une pression de compression sur la bande de papier (W) passant entre le rouleau en métal (16) et le rouleau en résine (18) et
les conditions de traitement incluent des conditions concernant la température de rouleau de l'ensemble de rouleaux (14) et la pression de compression et
la température de rouleau est choisie dans la plage allant de 25 à 160 °C, et
la pression de compression est choisie dans la plage allant de 3 à 10 N/mm.

2. Procédé de fabrication de papier à cigarettes (CP) selon la revendication 1, dans lequel
les conditions de traitement incluent une condition concernant la dureté du rouleau en résine (18).

3. Procédé de fabrication de papier à cigarettes (CP) selon la revendication 2, dans lequel la charge est une substance qui augmente non seulement la brillance, mais également l'opacité du papier à cigarettes (CP).

4. Cigarette comprenant du papier à cigarettes (CP) ayant une brillance supérieure ou égale à 10 %, mesurée selon la norme JAPAN TAPPI N°72,
dans laquelle le papier à cigarettes (CP) est fabriqué en satinant une bande de papier (W) contenant une charge pour augmenter la brillance, le papier à cigarettes (CP) présente une épaisseur de 20 à 100 µm et
la charge inclut du carbonate de calcium et,
la charge est contenue dans la bande de papier (W) dans la quantité dépassant au moins 10 gsm, et la bande de papier (W) présente un poids de base allant de 40 à 63 gsm.

5. Cigarette selon la revendication 4, dans laquelle le papier à cigarettes (CP) présente une opacité supérieure ou égale à 82.

6. Cigarette selon la revendication 4, dans laquelle le papier à cigarettes (CP) présente un lissé supérieur ou égal à 400".
